

# United States Patent Office.

E. H. ASHCROFT, OF BOSTON, MASSACHUSETTS.

*Letters Patent No. 81,576, dated September 1, 1868.*

## IMPROVED NON-CORROSIVE VALVE-SEAT.

*The Schedule referred to in these Letters Patent and making part of the same.*

TO ALL WHOM IT MAY CONCERN:

Be it known that I, E. H. ASHCROFT, of Boston, in the county of Suffolk, and State of Massachusetts, have invented new and improved Non-Corrosive Compositions of Metals for Valves for Steam-Boilers; and I do hereby declare that the following is a full, clear, and exact description thereof.

The object of my invention is to provide such metals or compositions of metals, to be used in the manufacture of safety-valves, or other valves for steam-boilers, as will not become corroded by the action of water, steam, air, nor by any other action to which such valves are exposed.

It is well known to engineers, and others, that many if not all of the safety-valves now in common use frequently become corroded to such an extent that the valve itself adheres to or is cemented to the "seat" so strongly that the whole object of such valves is defeated, and great danger to life and property ensues.

My invention consists in making these valves from the following non-corrosive alloys or metals, any and all of which answer the purpose more or less perfectly:

First, an alloy of nickel and copper, free from zinc.

Second, aluminum, alone or alloyed.

Third, an alloy of gold or silver.

Fourth, combinations of the above.

I prefer, sometimes, to make the valve itself of one composition or metal, and the "seat" of another, and, in the choice of the metal to be used, am governed somewhat by the exposure to which the valve will probably be subjected.

I do not confine myself to any exact proportions in casting these alloys, but, to enable others skilled in the art to make use of the first one mentioned, will state that I have found an alloy containing from twenty-five to fifty per cent. of nickel, with from fifty to seventy-five per cent. of copper, (entirely free from zinc,) to be non-corrosive, and admirably adapted to this purpose.

Having thus described my invention, I claim as new, and desire to secure by Letters Patent—

1. An alloy of nickel and copper, in any proportions, as set forth, for the construction of valves or valve-seats for steam, &c.
2. An alloy of gold or silver, in any desired proportions, for the construction of valves or valve-seats for steam, for the purpose set forth.
3. An alloy of aluminum, or aluminum alone, for the construction of valves or valve-seats for steam, for the purpose set forth.

E. H. ASHCROFT.

Witnesses:

CHARLES E. ASHCROFT,  
EDWIN J. WRIGHT.